

## UNITED STATES PATENT OFFICE

WILHELM SCHÄFER, OF BOCHUM, GERMANY

## TREATMENT OF COMPLEX ORES BY FLOTATION

No Drawing. Application filed September 18, 1929, Serial No. 393,584, and in Germany September 22, 1928.

The invention relates to the treatment of complex ores containing sulfides of zinc in the presence of other metalliferous sulfides such as lead or copper sulfides where the collective affinity of oils and similar substances is utilized to make a separation, especially to the so called froth flotation process in which the substances adhering to the oil are separated from the pulp by the use of a gas (such as air) in form of a froth. In these processes it is known to influence the floatative qualities by the use of reagents in addition to the oils. These known reagents, such as cyanide of potassium, sulfides and sulfites of alkali, are known to influence the floatative qualities, so that for instance it is possible to first separate the lead- or copper sulfide in the froth and to separate subsequently after having compensated the action of these reagents, and adding other reagents, the zinc sulfides in the froth. The action of the reagents, having the effect to keep down certain sulfides, is commonly known as depressing action while those reagents which compensate the action of the reagents of the first-mentioned kind, and effect the separation of the depressed mineral, are called anti-depressing reagents.

It has been found that a very effective depressing action on the zinc sulfides and at the same time an activating effect on the copper or lead sulfides, is produced by the addition of salts of the "hyposulfurous acid", that is of hyposulfites of the formula:



in which formula  $R_1$  and  $R_2$  may be either the same or different metals.

These hyposulfites are to be clearly distinguished from the thiosulfates of the formula  $R_2S_2O_8$  which are sometimes erroneously called also hyposulfites. The complex hyposulfites, especially those in which  $R_1$  is an alkali metal and  $R_2$  a base metal, are generally more effective as depressors of the zinc mineral while the simple salts in which  $R_1$  and  $R_2$  are the same metals, are generally more effective as activator of the lead and copper minerals.

In numerous cases it is of advantage to use hyposulfites in the presence of other reagents which liberate OH-ions or H-ions in the pulp; it may be useful to add these reagents together with the hyposulfites or before or afterwards. The hydroxyl ions may be furnished by bases or by salts having an alkaline reaction or by any compounds either organic or inorganic which in the process give rise to an alkaline reaction. The hydrogen ions may be furnished by acids or salts having an acid reaction or by compounds either organic or inorganic which in the process give rise to an acid reaction. When the reagents which liberate hydroxyl or hydrogen ions are added after the treatment of the pulp with the hydrosulfites, they assist in the reactivating of the blende, and allow the flotation of the zinc sulfide previously separated from the pulp.

The principal advantage of the hyposulfites over other known reagents of the depressing type, consists in the fact that the hyposulfites do not only depress the flotation of the zinc mineral, but at the same time do materially influence the floatative qualities of for instance the lead and copper sulfides. They have the further advantage that they are practically non-poisonous as contrasted to some other reagents used in the art. Some examples are given herewith to demonstrate the effect of the hyposulfites in comparison with cyanide of alkali frequently used.

## Example No. 1

100 gr. of a lead-zinc complex ore with quartzitic gangue were ground to 100 mesh fineness and diluted with four parts of water.  $\frac{1}{2}$  gr. of a hyposulfite of the following formula  $(Na_2Zn)(S_2O_4)_2$  were added and 1.5 gr. sodium silicate, furnishing hydroxyl ions, and several drops of a hard-wood tar oil and a pine oil were added. Then separation was made by producing a froth through the introduction of air under pressure and the following products were obtained:

|                                    |          |         |
|------------------------------------|----------|---------|
| 3.5 weight % lead-concentrate with | 71.4% Pb | 5.4% Zn |
| 98.5 weight % zinc residues with   | 0.6% Pb  | 9.4% Zn |
| 100.0 weight % heads with          | 3.1% Pb  | 8.2% Zn |

The zinc residues were not further treated 100

as the test should only demonstrate the activating action of the hyposulfites on the lead, and the depressing action on the zinc.

A parallel test was made in exactly the same manner and with exactly the same amount of ore but using 0.3 gr. sodium cyanide and 0.5 gr. zinc sulfate instead of the hyposulfite. The following products were obtained:

|    |                                    |          |         |
|----|------------------------------------|----------|---------|
| 16 | 3.7 weight % lead concentrate with | 60.5% Pb | 8.5% Zn |
|    | 96.3 weight % zinc residues with   | 0.8% Pb  | 9.2% Zn |
|    | 100.0 weight % heads with          | 3.0% Pb  | 9.2% Zn |

*Example No. 2*

15 A very complex and finely disseminated lead-zinc ore was ground to all-below 200 mesh and a test with 1000 gr. of this ore diluted in 4 parts of water was made. 0.6 gr.  $\text{Na}_2\text{S}_2\text{O}_4$  and 2 gr.  $\text{Na}_2\text{SiO}_3$ , furnishing hydroxyl ions, were added and also some drops, 20 of pine oil creosote and zanthate. The following products were obtained:

|    |                                    |          |          |
|----|------------------------------------|----------|----------|
| 25 | 9.5 weight % lead concentrate with | 57.8% Pb | 13.0% Zn |
|    | 9.1 weight % lead middlings with   | 25.2% Pb | 28.0% Zn |
|    | 81.4 weight % zinc residues with   | 3.8% Pb  | 17.2% Zn |
|    | 100.0 weight % heads with          | 10.9% Pb | 17.8% Zn |

30 A parallel test was made in exactly the same manner as before but using instead of the hyposulfite, 0.5 gr. sodium carbonate and 0.3 gr. cyanide of sodium and 0.4 gr. zinc sulfate. The following products were obtained:

|    |                                    |          |          |
|----|------------------------------------|----------|----------|
| 35 | 7.0 weight % lead concentrate with | 28.8% Pb | 17.9% Zn |
|    | 14.6 weight % lead middlings with  | 21.9% Pb | 18.5% Zn |
|    | 78.4 weight % zinc residues with   | 7.2% Pb  | 17.7% Zn |
|    | 100.0 weight % heads with          | 10.9% Pb | 17.8% Zn |

Having thus described my invention what I claim to protect is:

1. The step in the froth flotation process of treating finely divided zinc sulfides ore in the presence of other metalliferous ores to effect a separation of the zinc sulfide mineral from the other minerals which comprises treating the ores with a flotation solution containing a metal salt of the "hyposulfurous acid" of the formula  $\text{H}_2\text{S}_2\text{O}_4$ , and subjecting the ore pulp to flotation whereby the zinc sulfides to be separated are prevented from adhering to the froth.

2. The step in the froth flotation process of treating finely divided zinc sulfides ore in the presence of other metalliferous ores to effect a separation of the zinc sulfide mineral from the other minerals which comprises treating the ores with a flotation solution containing a complex metal salt of the "hyposulfurous acid" of the formula  $\text{H}_2\text{S}_2\text{O}_4$ , and subjecting the ore pulp to flotation whereby the zinc sulfides to be separated are prevented from adhering to the froth.

3. The step in the froth flotation process of treating finely divided zinc sulfides ore in the presence of other metalliferous ores to effect a separation of the zinc sulfide mineral from the other minerals which comprises treating the ores with a flotation solution containing a

metal salt of the "hyposulfurous acid" of the formula  $\text{H}_2\text{S}_2\text{O}_4$  and substances containing hydroxyl ions, and subjecting the ore pulp to flotation whereby the zinc sulfides to be separated are prevented from adhering to the froth.

4. In the froth flotation process of treating finely divided zinc sulfides ore in the presence of other metalliferous ores to effect a separation of the zinc sulfide mineral from the other minerals which comprises treating the ores with a flotation solution containing a complex metal salt of the "hyposulfurous acid" of the formula  $\text{H}_2\text{S}_2\text{O}_4$  and substances containing hydroxyl ions, and subjecting the ore pulp to flotation whereby the zinc sulfides to be separated are prevented from adhering to the froth.

5. The step in the froth flotation process of treating finely divided zinc sulfides ore in the presence of other metalliferous ores to effect a separation of the zinc sulfide mineral from the other minerals which comprises treating the ores with a flotation solution containing a metal salt of the "hyposulfurous acid" of the formula  $\text{H}_2\text{S}_2\text{O}_4$  and substances containing hydroxyl ions, whereby the zinc sulfides to be separated from the ore are prevented from adhering to the froth and thereafter adding to the solution a substance having hydrogen ions whereby the flotation of the zinc sulfides is permitted.

6. The step in the froth flotation process of treating finely divided zinc sulfide ore in the presence of other metalliferous ores to effect a separation of the zinc sulfide mineral from the other minerals which comprises treating the ores with a flotation solution containing a complex metal salt of the "hyposulfurous acid" of the formula  $\text{H}_2\text{S}_2\text{O}_4$  and substances containing hydroxyl ions and subjecting the ore pulp to flotation, whereby the zinc sulfides to be separated from the ore are prevented from adhering to the froth and thereafter adding to the solution a substance having hydrogen ions whereby the flotation of the zinc sulfide is permitted.

DR. WILHELM SCHÄFER.